

April 28, 1953

R. H. SAVAGE

2,636,838

# METHOD OF PRODUCING A FLAT MOISTUREPROOF PAPER LAMINATION

Filed April 14, 1947



BY

*INVENTOR.*

Marshals Biobel  
ATTORNEYS

## UNITED STATES PATENT OFFICE

2,636,838.

## METHOD OF PRODUCING A FLAT MOISTUREPROOF PAPER LAMINATION

Russell H. Savage, Chillicothe, Ohio, assignor to  
The Mead Corporation, Chillicothe, Ohio, a  
corporation of Ohio.

Application April 14, 1947, Serial No. 741,239

10 Claims. (Cl. 154—138)

1

This invention relates to a moistureproof paper lamination and the manufacture thereof, and more particularly to a lamination comprising two layers of paper and an interlayer of wax, and to methods of producing such a lamination.

It is an object of this invention to provide a method for producing a flat moistureproof paper lamination having a mineral coating on one side thereof suitable to receive high quality printing and having an ease of handling and utility in printing and forming operations comparable to that of a single unlaminated sheet of coated-one-side paper.

It is a further object of this invention to provide a method of laminating a sheet of coated-one-side paper to a sheet of paper by a moistureproof interlayer of wax so that the wax is confined substantially between said sheets of paper and the resulting lamination lies flat and has essentially the characteristics of a single sheet of coated-one-side paper in so far as printing and folding operations are concerned.

It is also an object of this invention to provide such a method for laminating two webs together by a continuous process in which the moisture contents of, and the tensions on, the webs leading into the laminating nip, as well as the pressure existing at the nip, are controlled so that a balanced stress relation between the webs is produced to provide for the production of a lamination free from objectionable curling tendency.

It is a further object of this invention to provide a moistureproof paper lamination having a mineral coating on one side thereof which lies flat without objectionable curling in use, and which has an appearance and ease of handling in printing and forming operations comparable to that of a single unlaminated sheet of coated-one-side paper.

Other objects and advantages of this invention will be apparent from the following description, the accompanying drawings, and the appended claims.

In the drawings—

Fig. 1 is a diagrammatic view in side elevation showing an apparatus suitable for applying wax-resistant size to paper in the practice of this invention;

Figs. 2 and 2a are diagrammatic views in side elevation of an apparatus suitable for producing laminations in accordance with this invention, the line A—A, which appears at the right and left ends of Figs. 2 and 2a respectively, indicating the line of division between two portions of

2

the continuous apparatus, for purposes of illustration herein; and

Fig. 3 is a detail of a doctor bar used in the apparatus of Fig. 2.

5 Mineral coatings are applied to a paper to improve the appearance by providing high gloss and whiteness, and are particularly desirable in the case of paper which is to receive printing, as the coating improves the printing characteristics of the paper and provides a better background for the inked impression. Such mineral coatings are commonly composed of a highly refined, finely divided white mineral material, such as clay or a natural or synthetic paper coating 10 mineral pigment, such as calcium carbonate, and an adhesive or bonding agent to bind the mineral coating material to the paper such as starch or casein. The coating material is usually applied to normally dried paper as a water suspension 15 by suitable means and the coated paper is further dried and then preferably calendered to produce the desired finish upon the surface of the layer or film of coating.

While it is common practice to apply mineral 20 coating to both sides of the paper—e. g. such paper as used in the printing of magazines containing high grade half-tone and multi-color reproductions, there are many fields of use in which it is desirable to coat only one side. Such paper is designated generally as coated-one-side paper. As is known in the art of making coated paper, coating only one side of paper tends to produce unbalanced conditions which cause the paper to 25 wrinkle or curl; and this tendency to curl, as 30 at the edges or into more or less irregular corrugations across the paper sheet or web are known to be affected by variations in moisture content or humidity. Curling is objectionable in subsequent handling steps, such as stacking sheets into 35 piles for shipment or handling by the user and is particularly objectionable in printing and machine forming operations, and particularly where stacks of sheets are used. A method of producing a non-curling coated-one-side paper is described in the patent to Donald F. Morris et al., 40 No. 2,314,797, assigned to the assignee of the present invention.

Under this invention paper having the printing 45 characteristics of coated-one-side paper is provided which paper in addition is adequately resistant to the penetration of moisture to meet commercial standards and requirements and which can be readily handled at the paper manufacturing plant, during shipment, and on printing and folding machines. In this invention the

moistureproofing of the paper is accomplished by the application of wax, such wax coating being applied to the uncoated side of coated-one-side paper for this purpose and as hereinafter described as a laminating or bonding layer. With the waxes ordinarily used in the waxing of papers, an uncovered or untreated waxed surface could be too slippery when cold and objectionably tacky when hot. A stack of such sheets could be unpredictably difficult if not impossible to handle since the individual sheets under certain temperature and pressure conditions would tend to stick together and form an unmanageable block of paper and, under other temperature conditions might slip over each other and over the press handling mechanisms so easily that a slight pressure would cause the whole stock to slide apart and scatter about the work room, making it quite difficult to keep the sheets stacked properly for transporting them, and difficult or impossible to handle them properly on printing or folding machines. Furthermore the usual waxes are quite penetrative when melted and would penetrate or strike through the ordinary coated-one-side paper and spoil the appearance and printability of the mineral coated surface unless specially prevented from doing so.

According to this invention it has been found that a satisfactory moisture resistant coated paper, which avoids the above difficulties, may be produced by forming a film of molten wax on a carrier sheet of wax resistant paper, cooling the wax below its applied molten temperature to an adequately non-flowing but heat-softened tacky condition, and laminating the wax-coated carrier sheet and the uncoated side of the coated-one-side paper to provide an interposed bonding wax film adequate to form an interlayer which is sufficiently moisture resistant to be generally termed moistureproof. It is important to so control the operation that the carrier sheet is not penetrated by the wax, in order to avoid the above mentioned difficulties in the transportation and use of sheets having waxy surfaces. It is usually desirable for the carrier sheet to be thin so that the laminated product will be thin enough to be handled comparably to suitably usable unlaminated coated-one-side paper. As the exposed surface of the "waxing" backing sheet or web should have such slip free surface characteristics that it may be handled like other used printing paper sheets, it has been found that the wax coating should be prevented from striking through and herewith that this can be accomplished with ordinary uncoated, machine finished, paper by applying a wax resistant size to the paper to be coated, and by causing the wax coating to assume a non-flowing condition, as by proper temperature control, immediately after the coating is applied to the paper.

In attempting to produce such a laminated sheet or web which will lie flat in use, substantial difficulties arise due to the dissimilarities of coated-one-side paper and said sized paper. These dissimilarities are increased or made more unpredictable by the effect of the hot wax in driving off moisture from the sized paper. This tends to produce unbalanced stress relations between the sides of the waxed paper and also between the webs which make up the finished lamination. This has presented great difficulties as resultant uncoordinated curling of each web of the laminated papers may occur and the effect may be additive or subtractive or more

or less neutralizing each other. I have found that this will cause unpredictable curling effects unless the laminating conditions are carefully controlled, and that such control is provided by the practicing of this invention, in which by regulating the relative moisture contents of the webs, the over-all and localized tensions on the webs as they are laminated, the laminating pressures and the relative driving speeds effective on web surfaces, such are avoided.

In the making of the laminated webs according to this invention to produce commercially satisfactory products the laminating material should be of such character that under the temperatures, heat and other conditions encountered in the manufacturing of envelopes or like products, or in the use thereof, the bending, folding, scoring, sealing, etc., of the products can be satisfactorily and effectively performed without disrupting the product as a whole or any of its constituent material, including the laminating material or adhesive, or without adversely affecting them for the intended use. For lower temperatures, sharp folds or creases, and less disruptive or adverse effects, so-called microcrystalline waxes have given quite satisfactory results. Microcrystalline waxes of varying characteristics are used, and generally speaking they are more flexible, less likely to break or crack, and more satisfactory as a laminating adhesive than the larger crystalline form of paraffin wax. Various laminating materials of varying characteristics are natural products in commercial use, and paraffin and microcrystalline waxes of varying characteristics are also produced in the petroleum and other industries, and similar or equivalent resinous adhesive or laminating materials likewise are found in nature and are produced synthetically. The characteristics of those which are readily available are usually readily ascertainable, or specified, and also they are made or modified to meet desired specifications. While so-called microcrystalline waxes have been found quite satisfactory in making the illustrative laminated paper for the manufacture of envelopes, as herein described, other materials of equivalent characteristics in laminating operations and subsequent manufacturing and usage may be used, and the precise specific characteristics of the wax or laminating material as herein referred to are not necessary to be more specifically stated.

Referring to Fig. 1, which illustrates a preferred apparatus embodying and for practicing the invention, the installation is shown somewhat diagrammatically, in connection with a paper making machine and arranged, as so illustrated, for applying a wax resistant size to the travelling paper web, as in a "tub sizing" operation during the production of paper on a paper machine. The size is applied at a point about two-thirds of the way through the drier section of the conventional paper machine, one section of drying rolls being indicated generally at 10 and another at 11. A web of paper 12 passes from the drying rolls 10 around a guide roll 13, through the nip of a pair of size press rolls 14 and 15, which apply the size to the paper, over guide rolls 16 and 17 and to drying rolls 11 proceeding thence through the drying and calendering operations usually performed on a conventional paper making machine. Roll 13 is spring mounted to maintain proper tension on the paper web 12 as it passes through

the size press rolls. Roll 16 has grooves cut in its surface which spiral outwardly from the center and function to keep the paper web stretched transversely. Such a roll is commonly called a worm roll. Roll 17 is also a worm roll, and is spring mounted to keep a uniform tension on the paper web.

The size press roll 15 dips in a pool of size maintained in tank 18, carrying a film of size on its surface and applying it to the paper web passing through the nip of the two size press rolls. Roll 15 carries an excess of size to the nip and the pressure between the rolls meters the proper quantity through the nip with the paper. Size may also be applied to the upper surface of the paper web, being supplied through a shower pipe 19 onto the surface of the paper just before the nip. An excess is supplied which forms a pool at the nip and the pressure between the rolls meters the proper quantity through the nip with the paper. A doctor blade 20 is provided to keep the surface of roll 14 clean. In order to supplement the action of the size press rolls in distributing the size uniformly across the paper web, it may be desirable to provide a spreader 21 between guide rolls 16 and 17.

A preferred formula for wax resistant size is 250 parts of methyl cellulose of medium low viscosity, 700 parts of an oxidized starch such as "Stayco," 440 parts of a dextrose corn sugar such as "Sweetose" as a plasticizer, and sufficient water to make a solution of about 8% solids content. The weight of the finished sized paper may desirably be about 26 pounds for 3,000 square feet, and conditions of application should be controlled so that about 1 to 1½ pounds of size (dry weight) are applied per 3,000 square feet. Application of such size will usually increase the resistance of the paper by about four times in the standard grease resistance test using mineral oil at 100° F.

Referring to Fig. 2, paper carrying a wax resistant size, prepared as described above, is unwound from the roll 30 supported on a conventional unwind stand 31. The web of paper 32 is led from roll 30 at a speed of about 300 feet per minute around idler guide rolls 33 and 33a, over idler guide roll 34, around a driven web feeding roll 35, around an idler roll 36, and over a wax-applying roll 37. Braking means 38 are provided to act on the roll 30 at the unwind stand to assist in maintaining proper tension on the paper web. The means shown comprise the brake band 39 frictionally engaging the brake drum 40 attached to the roll shaft, one end of the brake band being fixed and the other end being attached to the lever arm 41 near the pivot point 42 of the arm. The opposite end of the lever arm is adjusted by screw means 43 to tighten the brake band 39 as desired. Roll 36 is provided with similar braking means (not shown). Roll 35 is driven by a motor 44 through driving means, indicated diagrammatically at 45 in Fig. 2, providing for variable speed control, and a surface such as rubber is provided on the roll to grip the paper web. The tension on the paper web passing through the subsequent operations is principally controlled by the speed of this roll 35.

Wax-applying roll 37 is made of metal, such as chilled iron or steel, and dips in a pool of molten wax 46 contained in tank 47. A heater, indicated diagrammatically at 48, is provided to melt the wax. This heater is preferably electrical, and is provided with suitable temperature

controls to maintain the wax at a constant temperature. The roll 37 is driven by motor 49 through driving means 49a providing for a variable speed control which may be varied independently of the speed of roll 35, and is driven at a surface speed which is controlled with relation to the speed of travel of the paper web so that a slight excess of molten wax is picked up by roll 37 and applied to the paper web as the web passes over its surface. A doctor 50 is provided to smooth the wax on the paper and doctor off the excess, which excess wax drops back into the tank 47. This doctor is shown in more detail in Fig. 3. It comprises a bar 51, which may have a diameter of about ¼", and which has fine wire 52 wrapped in a close spiral around its surface. The bar 51 is supported by bearings such as 53, and is provided with the sprocket wheel 54 at one end which is slowly rotated by sprocket chain driving means 55 connected to motor 56 through a suitable speed reducing mechanism. The diameter of the wire 52 determines the thickness of the film of wax left on the paper web 32, since substantially the only wax passing the doctor is the wax which passes through the spaces between the wires. The wax, being molten, flows together again after passing the doctor to form a uniform even film. The rolls 35, 36 and 37, the motors 44, 49 and 56, the tank 47, and the doctor bar 50 may all be suitably supported by end pieces 60, located on each side of the paper web and supported by a pedestal 61, which also supports the heater 48.

The molten wax would soon penetrate the paper web if the wax were not quickly cooled below its melting point, even though the paper has been sized to greatly retard the rate of penetration. In order to cool the wax a stream of air is blown onto the paper through the duct indicated at 65 in Fig. 2. This duct extends across the width of the paper web and may conveniently be connected into the ventilating system usually provided in paper mills. The air is directed onto the uncoated side of the paper web so that there will be less chance for particles of dirt to be caught in the hot wax. The paper is guided from the wax-applying roll 37 into proper position just beneath the duct 65 by passing beneath a guide roll 66 and then passes beneath a guide bar 68. The wax is only cooled sufficiently to solidify it to a non-flowing condition and is left in a heat-softened tacky condition so that it may be readily bonded to the coated-one-side paper.

The wax applied to the sized paper is preferably a wax derived from petroleum which is commonly designated as microcrystalline wax. Microcrystalline wax has the desirable property of being soft enough to be flexible at room temperature and yet has a sufficiently high melting point so that it will not be unduly softened under any normal conditions of use to which laminations of the type disclosed herein are subjected. Preferably a microcrystalline wax is used which has a so-called melting point, as defined by standard test methods, of about 150 to 160° F. The wax is applied to the paper web at a temperature about 5° to 10° F. higher than its melting point.

After being cooled, the wax-coated paper web passes directly from guide bar 68 through a pair of laminating press rolls, the upper roll being indicated at 70 and the lower roll at 71. These rolls may conveniently be about 16" in diameter. The upper roll 70 should be provided with an

elastically yielding surface, such as a rubber cover of about 50-75 Pusey and Jones hardness, and the lower roll 71 should have an unyielding surface, such as chilled iron or steel. The rolls 70 and 71 may suitably be journaled in end pieces 52, located on each side of the paper web and supported on a pedestal 73. The rolls are individually driven by variable speed motors 74 and 75, motor 74 driving the upper roll through driving means 77 and motor 75 driving the lower roll through driving means 78. A girder 79 provides a support for these motors.

A roll of coated-one-side paper is indicated at 80. This may suitably weigh about 53 pounds per ream of 25" x 38" sheets, of which weight 15 8 pounds may be the mineral coating. This coated paper may be produced as described in the above mentioned patent to Morris et al., No. 2,314,797. The roll of paper is supported on a conventional unwind stand 81 provided with wheels 82 which roll on tracks 83, so that the stand 81 may be rolled to one side of the apparatus for placing new rolls of paper in position. The web 84 of coated-one-side paper is led from the roll 80 around a guide roll 85 and guide bar 86 and onto the surface of the laminating roll 71, and travels with its coated surface in contact with roll 71 into the nip with the upper laminating roll 70. Guide bar 86 exerts a drag on the paper to feed the web to the roll 71 under sufficient tension so that it will lie smoothly on the roll surface. An additional control on the tension is provided by braking means 88 on the unwind stand 81, which is similar in construction and operation to braking means 38 on unwind stand 31. The wax-coated, sized paper web 32 is led into the nip with the uncoated side in contact with roll 70 so that the heat-softened wax coating is applied to the uncoated side of the coated-one-side paper.

The laminating nip between rolls 70 and 71 functions to cause the wax coating on the sized paper to conform to surface irregularities of the coated-one-side paper and to cause the wax to penetrate between the surface fibers of the paper sufficiently to produce a firm bond over the entire surface. This is accomplished by providing a yielding rubber cover on roll 70 which will conform to irregularities in the thickness of the wax-coated sized paper, and by providing sufficient pressure between the rolls to cause the rubber cover to be deformed and provide a nip of considerable area. The weight of roll 70 will be sufficient for this purpose if it is substantially solid and made of iron or steel with the exception of the rubber cover. One or both of the rolls 70 and 71 may be slightly crowned, i. e., the diameter increased toward the middle, and to the extent desired to offset axial bending resulting from the pressure or weight of the rolls, so that the pressure can be kept uniform along the nip.

In practice it has been found that the pressure between the rolls must be carefully controlled to produce a lamination which will lie flat in use. When the pressure was above a proper value it was observed that the lamination would curl transversely, the sides of the lamination tending to curl upwardly. When the pressure was below such value the sides of the lamination would tend to curl downwardly. When the pressure was greater at one end of the rolls than at the other end, one side of the lamination would curl upwardly and the other side of the lamination would curl downwardly. To provide close control of the pressure, each

5 end of the upper laminating roll 70 is journaled in adjustable bearings provided with an adjustable screw means, indicated at 90, for moving each end of the roll up or down. The screw means are adjusted during operation until the lamination produced is flat in a transverse direction.

10 The tendency toward curling as above described is believed to result from a stretching of the lamination in the nip of the laminating rolls. The rubber cover of the upper roll 70 is deformed in a circumferential direction by the pressure applied by the lower roll 71. If the pressure is not equally distributed along the nip the rubber will be deformed more where the pressure is greater. The lamination passing through the nip will be gripped more firmly by the rubber than by the metal surface of roll 71 and will be stretched as the rubber is deformed. If the pressure is not equal along the nip between the rolls, the lamination will be stretched to a greater extent where the pressure is greater, causing the curl described. Thus, in the case of rolls which are crowned to compensate for bending, when the pressure between the rolls is correctly correlated with the crown provided on one or both of rolls 70 and 71, the crown will just offset bending of the rolls and the pressure between the rolls will be equal along the nip. At lesser pressures the rolls will not bend as much as is provided for by the crown and the pressure between the rolls will be greater in the middle than at the ends. When the pressure is greater than the correct pressure, the rolls will be bent too much for the crown provided and the pressure between the rolls will be greater at the ends than in the middle.

15 In order to produce a lamination which is free from curl in a longitudinal direction it has been found that the tension on the paper webs passing to the laminating nip between rolls 70 and 71 should be carefully controlled, and the relative speeds of rolls 70 and 71 should also be carefully controlled. During the time that longitudinal tension is applied to a paper web, the web is stretched longitudinally by an amount dependent upon the amount of tension. When the tension is removed an elastic recovery takes place, the web shrinking longitudinally to regain its original dimension at least in part. If, for example, the upper sized web 32 is stretched more than the lower mineral coated web 84 as the webs are laminated together, web 32 will subsequently tend to shrink more than web 84, tending to cause the lamination to curl upwardly in a longitudinal direction toward the web 32. Such a curl may be corrected by reducing the tension on the web which is being stretched too much, or by increasing the tension on the other web. The tension on web 32 is controlled by the speed of the feeding roll 35 relative to the speed of the laminating rolls, and by the amount of drag exerted by the braking means on rolls 30 and 36. The tension on web 84 is controlled by the amount of drag exerted by the braking means on roll 80. The speeds of laminating rolls 70 and 71 relative to each other provide an additional control of the amount of stretch given the paper webs at the time they are laminated together. In practice, the above mentioned controls should be maintained in proper correlated relationship to avoid such an unequal stretching of the one web with respect to the other web that the lamination would tend to curl longitudinally.

20 25 30 35 40 45 50 55 60 65 70 75 80 85 90 95 In order to produce a lamination which will

In flat in use it is desirable that the two webs, as they are brought together to be laminated, be at approximately the same moisture content. If two webs having different moisture contents are laminated together and then come to equilibrium at the same moisture content, the web originally having a higher moisture content will shrink and the web having a lower moisture content will expand, causing the lamination to curl in the direction of the web which initially had the higher moisture content. The heat of the hot wax applied to the sized paper web 32, and the cooling air blown on the web through the duct 65, drive off moisture from this web. Therefore the moisture content of the sized paper as supplied to the wax coating step should be higher than the moisture content of the coated-one-side paper as supplied to the laminating step. This could be provided for by accurately controlling the moisture contents of rolls of paper to be used so that the moisture content of the roll of sized paper 30 is just enough more than the roll of coated-one-side paper 80 to offset moisture losses caused by the operation of applying and cooling the wax coating. However, this would present difficulties in the ordinary processes of manufacture, since both types of papers are ordinarily produced to have a moisture content of the order of about 5%, with a variation in moisture content of as much as 1% from roll to roll.

It has proven to be expedient to increase the moisture content of the sized paper as necessary at the laminating machine by adding moisture to it immediately before the wax coating operation. Steam is supplied through a pipe 91 provided with a narrow slot extending the width of the paper web. A galvanized sheet iron box 92 forms a chamber through which the paper web passes in contact with the steam. This box is of slightly greater width than the width of the paper web and is made sufficiently high for the paper to have time to take up the required amount of moisture by the time the paper web has passed through the box and out of a slot 93 at the top of the box. By controlling the flow of steam the required amount of moisture may be added to the paper web to produce a lamination which will be free of curl in use. Under the conditions of operation described it has been found that an increase of approximately 2% in the moisture content of the paper web will offset the loss of moisture caused by the hot wax and the cooling air, but control of the flow of steam may be judged satisfactorily by experience and observation of the lamination being produced.

From the laminating press rolls 70 and 71 the lamination passes over idler guide rolls 95 and 96 to a pair of metal cooling rolls 97 and 98. The cooling rolls are spaced apart slightly and geared together by gears 100 and 101 to rotate at the same speed, the lower roll 97 being rotated at the speed of the lamination by motor 102 through driving means 103. The rolls are about 24 inches in diameter, are hollow and are arranged so that cooling water may be circulated through them to keep the surface at about room temperature or a little below. The lamination passes first around most of the surface of cooling roll 97 and then the opposite face of the lamination passes most of the way around the surface of cooling roll 98. The lamination is thus cooled, first from one side and then from the other side, until the wax interlayer is cooled to about room temperature. At this temperature the wax is in a condition which will hold the

two paper webs firmly bonded together through normal handling conditions.

The laminated web continues on to a sheet cutter, shown diagrammatically in Fig. 2a, which cuts the web into sheets of the required size. A suitable number of spaced apart idler guide rolls 105, 106, 107, 108 and 109 conduct the web to slitters, indicated at 110, in proper position for slitting, and the web then passes through the nip between driven rolls 115 and 116, which feed the web through the cutter at the proper speed and maintain the web under proper tension for slitting. The rolls 115 and 116 are driven by a variable speed motor 117 through driving means 118, the speed of the motor being controlled by an automatic tension control indicated at 120. The tension control comprises an idler roll 121 mounted on the end of a pivoted arm 122, the arm being connected to a rheostat controlling the speed of the motor 117 in proper manner for movement of the end of the arm supporting the idler roll 121 to effect regulation of the speed of the motor. The idler roll 121 is arranged to press on the laminated web after the web has passed over guide roll 107 and before the web passes over guide roll 108, the arrangement being such that the web is under proper tension when there is a slight sag between rolls 107 and 108, due to the pressure of roll 121, and any increase or decrease in the amount of sag will cause the roll 121 to be lowered or raised, which in turn causes the supporting arm 122 to regulate the rheostat as necessary to increase or decrease the speed of rolls 115-116 and correct the web tension.

The slitters 110 are of the usual construction comprising rotary knives adapted to trim the edges of the web and may, in addition, slit the web longitudinally into required widths, as is understood in the industry. The web then passes from rolls 115-116 to a revolving knife cutter, indicated at 125, which cuts the web laterally between a revolving knife and a fixed knife bar to produce sheets. The length of the sheets is varied as required by adjusting the speed of revolution of the revolving knife relative to the speed of the web, and for this purpose the revolving knife is driven by motor 117 through driving means 126 providing variable speed control. The cut sheets fall onto lay boy tapes 130 which convey the sheets to a receiving box 131 where the sheets are stacked. The tapes are driven and supported by rolls 132, 133, 134 and 135, which are rotated by the motor 117 acting through a driving means 136.

A wind-up stand 140 is also shown in Fig. 2, and may be used to wind the laminated web into a roll when it is desired to cut the web into sheets at some later time. However, winding into a roll has been found to stretch the lamination unevenly unless the lamination has an extremely uniform caliper, the uneven stretching causing waviness or tendency to curl in the finished sheets. It is preferable, therefore, to produce the lamination and cut it into sheets in one continuous operation as described.

In accordance with this invention means are provided for continuously applying a moisture-proof coating to coated-one-side paper on a thin backing sheet so that the moistureproof coated-one-side paper may be handled in the usual manner in such operations as printing and forming. A process has been provided by which the lamination of coated-one-side paper and the protecting backing sheet may be produced which

## 11

will lie flat in use and be free from tendency to curl. Additionally the lamination will have an appearance and feel and ease of handling comparable to that of a single unlaminated sheet of coated-one-side paper, because the exposed surface of the backing sheet will have a surface similar to that of the uncoated surface of the coated-one-side paper, and the thickness of the lamination will not be objectionably greater than that of unlaminated coated-one-side paper.

While the process and product herein described constitute preferred embodiments of the invention, it is to be understood that the invention is not limited to this precise process and product, and that changes may be made therein without departing from the scope of the invention which is defined in the appended claims.

What is claimed is:

1. A method of producing a flat moistureproof paper lamination having a mineral coating on one side thereof suitable to receive high quality printing which comprises the steps, performed in a continuous manner, of applying a wax resistant size to a paper web, passing said web through a moisture laden atmosphere for a limited time for increasing the moisture content of said sized paper in excess of the moisture content of a coated-one-side paper web by an amount sufficient to offset loss of moisture from said sized paper in subsequent coating operations, applying a coating of molten microcrystalline wax to one side of said sized paper, immediately cooling said coating to a heat-softening condition below the melting point of said wax and eliminating moisture therefrom, pressing the wax-coated side of said sized paper onto the uncoated side of said coated-one-side paper under controlled uniform transverse pressure and uniform longitudinal tension producing a balanced stressed relation between said sized paper and said coated-one-side paper, and cooling said wax to produce a flat, evenly bonded lamination and the moisture contents of said webs being in such equilibrium that changes in atmospheric humidity produce substantially coextensive dimensional changes in both said webs.

2. A method of moistureproofing a sheet of paper having a mineral coating on one side thereof without interfering with its utility for such operations as printing and folding which comprises the steps, performed in a continuous manner, of applying a wax resistant size to a web of paper, passing said web into contact with steam for a limited time increasing the moisture content to a value greater than the moisture content of a web of coated-one-side paper, applying a uniform coating of molten microcrystalline wax to said sized paper, immediately cooling said coating to a heat-softened condition below the melting point of said wax and eliminating moisture from said sized web, said size and said cooling of the wax preventing said wax from striking through said paper, applying the heat-softened wax-coated surface of said sized paper web to the uncoated surface of said coated-one-side paper web while maintaining controlled uniform stress-producing longitudinal tension on said webs and uniform pressure across said webs, and while maintaining said moisture content of the webs and transverse and longitudinal tension applied thereto so regulated that a balanced stress relation between the webs is produced, and cooling said wax to produce a flat, evenly bonded lamination and the moisture contents of said webs being in such equilibrium that changes in atmospheric

70

75

## 12

humidity produce substantially coextensive dimensional changes in both said webs.

3. A method of producing a flat moistureproof paper lamination having a mineral coating on one side thereof suitable to receive high quality printing and having an ease of handling in printing and forming operations comparable to that of a single unlaminated sheet of coated-one-side paper which comprises the steps, performed in a continuous manner, of applying a wax resistant size to a thin sheet of paper and passing said sheet through a moisture laden atmosphere for a limited time increasing the moisture content of said sheet to a value greater than a sheet of coated-one-side paper, applying a uniform coating of molten wax to one side of said sized sheet, partially cooling said coating sufficiently to prevent the wax from striking through said sheet but leaving said wax in a heat-softened condition and eliminating moisture from said wax-coated sheet, bringing the uncoated surface of said sheet of coated-one-side paper having a moisture content substantially equal to the then moisture content of said wax-coated sheet against the heat-softened wax coating on said sheet, pressing said sheets together under controlled pressure across said sheets with controlled uniform stress-producing tension longitudinally of said sheets and cooling said wax to produce a flat, evenly bonded lamination and the moisture contents of said sheets being in such equilibrium that changes in atmospheric humidity produce substantially coextensive dimensional changes in both said sheets.

4. A method of producing a flat moistureproof paper lamination having a mineral coating on one side thereof suitable to receive high quality printing and having an ease of handling in printing and forming operations comparable to that of a single unlaminated sheet of coated-one-side paper which comprises the steps, performed in a continuous manner, of applying a wax resistant size to a thin sheet of paper and passing said sheet through a moisture laden atmosphere for a limited time increasing the moisture content of said sheet to a value greater than a sheet of coated-one-side paper, applying an excess of molten microcrystalline wax to said sized sheet, doctoring off excess wax to produce an even coating of predetermined thickness on said sheet, partially cooling said coating sufficiently to prevent the wax from striking through said sheet but leaving said wax in a heat-softened condition and eliminating moisture from said wax-coated sheet, bringing the uncoated surface of said sheet of coated-one-side paper having a moisture content substantially equal to the then moisture content of said wax-coated sheet against the heat-softened wax coating on said sheet, pressing said sheets together between a yielding elastic surface and an unyielding surface with controlled pressure across said sheets and controlled uniform stress-producing longitudinal tension, and cooling said wax to produce a flat, evenly bonded lamination.

5. A method of continuously producing a flat moistureproof paper lamination having a mineral coating on one side thereof suitable to receive high quality printing and having an ease of handling in printing and forming operations comparable to a single unlaminated sheet of coated-one-side paper which comprises the steps of continuously feeding to coating and laminating operations, a thin paper web which has been sized so that it resists the penetration of wax, said sized

## 13

web during said operations being passed through a moisture laden atmosphere for a limited time increasing the moisture content thereof to a value greater than a web of coated-one-side paper, continuously applying a coating of molten micro-crystalline wax to one side of said web, partially cooling said coating sufficiently to prevent the wax from striking through said web but leaving said wax in a heat-softened condition and eliminating moisture from said wax-coated web, continuously feeding said coated-one-side paper web having a moisture content substantially equal to the then moisture content of said wax-coated web onto said wax-coated web with the uncoated side next to said heat-softened wax coating, continuously rolling said webs together under controlled pressure across said webs while applying controlled tension longitudinally of said webs, and cooling said wax to produce a flat, evenly bonded lamination free of curl-producing unbalanced stresses.

6. A method of producing a flat moistureproof paper lamination having a mineral coating on one side thereof suitable to receive high quality printing which comprises the steps, performed in a continuous manner, of applying a wax resistant size to a thin paper web, passing said web through a moisture laden atmosphere for a limited time for increasing the moisture content of said sized paper in excess of the moisture content of a coated-one-side paper web by an amount of about 2%, applying a coating of molten micro-crystalline wax to one side of said sized paper, immediately cooling said coating to a heat-softened condition below the melting point of said wax, pressing the wax-coated side of said sized paper onto the uncoated side of said coated-one-side paper under controlled pressure across said webs while applying controlled longitudinal tension to said sized sheet, and cooling said wax to produce a flat, evenly bonded lamination free of curl-producing unbalanced stresses.

7. A method of producing a flat moistureproof paper lamination having a mineral coating on one side thereof suitable to receive high quality printing which comprises the steps, performed in a continuous manner, of applying a wax resistant size to a thin paper web, passing said web through a moisture laden atmosphere for a limited time causing the moisture content of said sized paper to exceed the moisture content of a coated-one-side paper web by an amount of about 2%, applying a coating of molten microcrystalline wax to one side of said sized paper, immediately cooling said coating to a heat-softened condition below the melting point of said wax, pressing the wax-coated side of said sized paper onto the uncoated side of said coated-one-side paper by passing said papers through the nip of a pair of laminating press rolls, the roll pressing on said sized sheet having a yielding elastic surface and the roll pressing on said coated-one-side paper having an unyielding surface, maintaining substantially uniform pressure between said rolls across said web to prevent curling in a transverse direction in the finished lamination and maintaining both said webs passing through said nip under substantially uniform tension to produce equivalent stresses therein for preventing curling in a longitudinal direction in the finished lamination.

8. A method of continuously producing a flat moistureproof paper lamination having a mineral coating on one side thereof suitable to receive high quality printing which comprises the steps of applying a wax resistant size to a thin paper

## 14

web, advancing said sized paper web in a continuous and progressive fashion under controlled uniform tension, applying steam to said advancing web to raise the moisture content thereof to exceed the moisture content of a coated-on-one-side paper web by an amount of about 2% sufficient to offset loss of moisture in the subsequent coating operation, applying a coating of molten microcrystalline wax to one side of said advancing web, cooling said coating to a heat-softened condition below the melting point of said wax, passing said advancing web under controlled uniform tension through the nip of a pair of rotating press rolls, the roll in contact with the uncoated side of said sized web having a yielding elastic surface and the other roll having an unyielding surface, continuously and progressively feeding said coated-one-side paper web through said nip with the uncoated side in contact with the heat-softened wax coating of said sized web, applying sufficient pressure between said press rolls to cause said yielding surface to be deformed at the nip and provide a nip of considerable area, maintaining substantially evenly distributed and uniform pressure along the nip to prevent curling of the finished lamination, and cooling said wax to produce a flat, evenly bonded lamination.

9. A method of producing a flat moistureproof paper lamination having a mineral coating on one side thereof suitable to receive high quality printing and having an ease of handling in printing and forming operations comparable to that of a single unlaminated sheet of coated-one-side paper which comprises the steps, performed in a continuous and progressive manner, of applying a wax resistant size to a thin web of paper and passing said web through a moisture laden atmosphere for a limited time increasing the moisture content of said sheet to a value greater than a web of coated-one-side paper, applying a uniform coating of molten wax to one side of said sized web, partially cooling said coating sufficiently to prevent the wax from striking through said web but leaving said wax in a heat-softened condition and eliminating moisture from said wax-coated web, bringing the uncoated surface of said web of coated-one-side paper having a moisture content substantially equal to the then moisture content of said wax-coated web, pressing said webs together between a yielding elastic surface and an unyielding surface with controlled uniform pressure across said webs while maintaining both of said webs under controlled uniform tension, cooling said wax to produce a flat, evenly bonded lamination, and cutting said lamination into sheets.

10. A method of producing a flat moistureproof paper lamination having a mineral coating on one side thereof suitable to receive high quality printing and having an ease of handling in printing and forming operations comparable to that of a single unlaminated sheet of coated-one-side paper which comprises the steps, performed in a continuous manner, of applying a wax resistant size to a thin web of paper and passing said web through a moisture laden atmosphere for a limited time increasing the moisture content of said web to a value, applying a uniform coating of molten wax to one side of said sized web, partially cooling said coating sufficiently to prevent the wax from striking through said web but leaving said wax in a heat-softened condition, bringing the uncoated surface of a web of coated-one-side paper having a moisture content substantially equal to the

15

then moisture content of said wax-coated web against the heat-softened wax coating on said wax-coated web, rolling said webs together under controlled uniform transverse pressure between a roll having a yielding elastic surface and a second roll having an unyielding surface, maintaining said webs under substantially uniform and equivalent stress-producing tension during said rolling, and cooling said wax to produce a flat, evenly bonded lamination, and cutting said lamination into sheets.

RUSSELL H. SAVAGE.

References Cited in the file of this patent

15

## UNITED STATES PATENTS

| Number    | Name | Date         |
|-----------|------|--------------|
| 1,473,096 | Hill | Nov. 6, 1923 |

16

| Number      | Name              | Date          |
|-------------|-------------------|---------------|
| 1,866,689   | Van Hamm-Wilshire | July 12, 1932 |
| 2,031,035   | Dreymann          | Feb. 18, 1936 |
| 2,031,026   | Dreymann          | Feb. 18, 1936 |
| 5 2,153,754 | Hodgdon           | May 16, 1939  |
| 2,360,277   | Robertson         | Oct. 10, 1944 |
| 2,402,903   | Massey et al.     | June 25, 1946 |
| 2,430,459   | Farrell et al.    | Nov. 11, 1947 |

## OTHER REFERENCES

"Microcrystalline Waxes and the Paper Industry" by John C. Dean, published in Paper Trade Journal, vol. 120, No. 7, February 15, 1945; pages 28-32.